

## UNITED STATES PATENT OFFICE

NORMAN D. HARVEY, JR., OF PITTSBURGH, PENNSYLVANIA, ASSIGNOR TO CARBIDE & CARBON CHEMICALS CORPORATION, A CORPORATION OF NEW YORK

## UNHAIRING BATH AND PROCESS OF TREATING HIDES

No Drawing.

Application filed March 21, 1930. Serial No. 437,942.

The invention relates to baths for unhauling hides. Such baths are useful in recovering wool or other hair for textile purposes, but their principal application is in the preparation of hides for tanning.

Hides are normally delivered at the tannery after curing by salting or sun-drying. At the tannery the hides are soaked to cleanse and rehydrate them. They are then unhaired, plumped, and finally tanned.

The unhauling and plumping operations, as a rule, are carried out together, as by treating the hides for two or three days in a bath prepared by suspending lime in water, and then adding sodium sulphide. Such a bath decomposes the epidermis, or outer layer of the hide; and since the epidermis lines the hair follicles and grips the hairs the latter are loosened so that they can be removed mechanically. At the same time the corium (which lies under the epidermis and forms the substance of the finished leather) swells, takes on a firmer texture, and is otherwise so modified that it becomes amenable to tanning. This effect is called plumping. An alkalinity represented by pH at least 10 is required for unhauling, but a higher alkalinity promotes the process. Plumping requires pH at least about 12, while 12.5 gives better results. If plumping proceeds too rapidly, so that it outstrips the disintegration of the epidermis, the corium closes on the roots of the hairs and prevents proper loosening of the latter.

In accordance with the invention, monoethanol amine is used as an unhauling agent. For example, the hides may be covered with an aqueous solution of monoethanol amine of such concentration that about one pound of amine is present for each 100 pounds of hides; but the proportion of amine to hides may be varied over a wide range. All dilute solutions of monoethanol amine have a pH value of 11.6 to 11.7.

Monoethanol amine has only a feeble

plumping action; and it may advantageously be used in conjunction with more strongly alkaline agents having pronounced plumping properties, such as the hydroxides or sulphides of the alkali and alkaline earth metals. Certain other amines, such as methyl amine and ethylene diamine have both plumping and unhauling properties and may be admixed with monoethanol amine. A bath containing the proportion of monoethanol amine mentioned above (one pound per hundred pounds of hides) with about 10 pounds of lime per hundred pounds of hides has very good unhauling and plumping properties.

Like known unhauling baths, those containing monoethanol amine increase in efficiency during use. This appears to be due to the incorporation of substances extracted from the hides. Among the substances which give rise to the increased efficiency, monoethanol amine sulphide formed by the interaction of the bath with hide proteins seems to be one of the most important.

When used in conjunction with lime, monoethanol amine promotes absorption of the lime by the hides. Hides treated with such a mixture are lighter in color, and have a finer and thicker grain than hides treated with the usual lime-sulphide compositions.

When wool is to be removed from sheepskins, a less alkaline bath, such as one containing monoethanol amine alone, may be used. Whereas the usual agents for this purpose dissolve the roots of the hairs, it is possible with monoethanol amine baths to loosen the hairs without destroying the root, or portion embedded in hide. The fibre length and poundage of the wool recovered are thus increased.

I claim:—

1. An unhauling bath containing monoethanol amine and a plumping agent.
2. An unhauling bath containing monoethanol amine, and an inorganic compound of alkaline reaction.

3. An unhairing bath containing mono-ethanol amine and lime.
4. An unhairing bath containing mono-ethanol amine and lime in the proportions of 5 approximately one pound to ten.
5. The process of treating hides to remove hair therefrom which consists in soaking the hides in a bath containing monoethanolamine until the hairs are loosened.
- 10 6. The process of treating hides to remove hair therefrom which consists in soaking the hides in a bath containing monoethanolamine and lime until the hairs are loosened.

15 In testimony whereof, I affix my signature.

**NORMAN D. HARVEY, JR.**

20

25

30

35

40

45

50

55

60

65